

Patented Jan. 9, 1923.

1,441,740

# UNITED STATES PATENT OFFICE.

AMOS NELSON, OF GLEDSTONE, WEST MARTON, NEAR SKIPTON, ENGLAND.

## MERCERIZING OF COTTON.

No Drawing.

Application filed November 7, 1921. Serial No. 513,317.

*To all whom it may concern:*

Be it known that I, AMOS NELSON, residing at Gledstone, West Marton, near Skipton, in the county of York, England, have invented 5 certain new and useful Improvements Relating to the Mercerizing of Cotton, of which the following is a specification.

This invention relates to the mercerizing of cotton and has for its object to carry out 10 this operation more efficiently and economically than can be done by any of the existing processes. In the ordinary way mercerization is carried out on yarns, in hank and warp form, and also on pieces, and no perfect method of mercerizing cotton in the 15 yarn and cloth has been arrived at up to the present owing to the fact that the amount of twist which the yarn contains prevents it from becoming fully impregnated with the 20 alkali, with the result that only the outer surface of the yarn becomes properly mercerized. It has been attempted to mercerize rovings in the form of hanks but the length put into a hank is so short and creates so 25 many knots or pieceings that yarns can only be produced at greatly increased cost and with many defects.

According to this invention in order to overcome these defects the cotton is subjected to the mercerizing process whilst it 30 is in the form of a rope or chain comprising a number of slightly twisted slubber or intermediate rovings, laid alongside of one another, and hereinafter referred to as rovings.

These rovings are arranged side by side to form a chain, stretch or sliver, and they are not twisted together upon the axis of the chain. As many rovings are thus placed 40 together as will enable the chain to have sufficient strength to withstand the tension required for mercerizing. As each roving remains separate in the chain, the mercerizing liquid can flow freely between the rovings, and can penetrate the material of all of them to an equal extent, which is not possible when the rovings are twisted together. Each roving contains only sufficient twist 45 to enable it to withstand the tension to which it is subjected during the mercerizing and washing process and to enable the caustic soda, or other alkali to penetrate to every fibre and so give a perfect mercerization of all the fibres, so that when the rovings are 50 subsequently spun into yarn, single yarn can be made just as bright as two-fold yarn.

For the purpose of the invention the rovings may be taken from a number of bobbins and be converted into a rope, or chain comprising any predetermined number of rovings. One or more of these chains arranged side by side are then passed in a state of tension through the caustic soda, or other alkali, and are then subjected to a washing and steaming process which removes all traces 60 of the alkali without resorting to the use of sulphuric acid for effecting the usual souring operation. After the chains have been subjected to the washing and steaming operation, they are subsequently dried and separated and are then ready for being converted into yarn.

The first process may consist in taking the sliver to a slubbing frame and imparting a sufficient number of turns to the slubber roving to prevent the fibres from shrinking in the process of mercerizing, or the roving may be taken from an intermediate frame or a jack frame; the first process however is preferable as it enables finer 75 counts to be spun, whereas the second process is more costly and eliminates one drawing operation with the result that the yarn is less even. As the various machines in a spinning factory are usually arranged in a 80 standardized order or sequence, a left hand twist is advantageously put into the rovings so that the slubbing frame can occupy its usual relative position. The bobbins on which the slubbing or intermediate rovings 85 are wound are now taken and put into a chaining machine adapted to hold a sufficient number of bobbins to form the chain, say for example, 24 to 100 bobbins. The chain may be allowed to coil into a can or be wound 90 on to a cheese or beam, the length of chain being determined by the length that can be got on to the bobbins, or by the length that is most suitable for spinning. The chains are now subjected to the mercerizing process 95 by passing them through caustic soda, which is preferably kept as nearly as possible at a temperature of 40° Fahrenheit. The chains are now subjected to a washing process which consists in causing them to 100 pass through boiling water and steam alternately a sufficient number of times to free them from caustic soda without resorting to the usual souring process. The chains are now subjected to a drying process and after 105 being dried may be again coiled into cans and taken to a machine which separates the

rovings in each chain and winds them on to bobbins. The latter are then taken to a machine which restores the rovings to their untwisted condition to enable them to be 5 drawn in the ordinary way.

By my present invention the rovings are never handled during the various processes and they come out so clean and soft after 10 being washed a number of times in boiling water and steam that the subsequent drawing operation can be done with ease. Single mercerized yarns can be made in nearly 15 every count from coarse to very fine, every fibre is mercerized, and a brightness can be obtained without the expensive method of 20 using two fold yarn. Very fine light and bright cloths can be made and by making single yarn cloths they are much lighter than the old two fold yarn cloths and effect 25 a great saving in the amount of cotton used. Owing to the fact that the caustic soda penetrates completely through the whole of the fibres the lustre and brightness will always remain however many times the cloth is 30 washed whereas when the material has been subjected to the mercerization process whilst in the state of yarn or cloth, and particularly cloth, the caustic soda does not penetrate all through the yarn and the inner fibres are not mercerized, consequently when the outer fibres wear away the cloth loses its lustre.

This objection as also the defects and increased cost which arise through mercerizing rovings in the form of banks are entirely overcome by mercerizing the slubber 35 and intermediate rovings in the form of a chain. By mercerizing the yarn whilst in the form of a chain, the cost of the mercerizing processes is considerably less and the subsequent cost and trouble in spinning is 40 reduced to a minimum. The same length that the spinner gives on the roving bobbin will be given back in one length and no more knots or piecings will be produced by this process than by ordinary spinning. Any 45 counts from coarse to fine can be spun out of rovings mercerized in accordance with this invention.

What I claim as my invention and desire to secure by Letters Patent in the United States is:—

A method of producing mercerized yarn, which consists in first arranging a number of rovings of slightly twisted yarn side by side to form a chain without twisting the 55 rovings together spirally on the axis of the chain, and then subjecting the chain of rovings to the mercerizing operation while under tension.

In testimony whereof I affix my signature. 60

AMOS NELSON.